

3,212,254

**TWO COMPONENT AMINE NITRATE MONOPROPELLANTS AND METHOD OF PROPULSION**  
 Homer M. Fox, Bartlesville, Okla., assignor to Phillips Petroleum Company, a corporation of Delaware  
 No Drawing. Filed Aug. 14, 1957, Ser. No. 678,243  
 17 Claims. (Cl. 60—35.4)

This application is a continuation-in-part of my copending application Serial No. 465,957, filed November 1, 1954, and my copending application Serial No. 542,515, filed October 24, 1955, said latter application now abandoned.

This invention relates to novel two-component monopropellant compositions suitable for use in rocket motors, ram-jets, pulse-jets and the like. In a further aspect, this invention relates to a method of operating such motors.

Rocket motors are operated by burning a mixture of fuel and oxidant in a combustion chamber and causing the resulting gases to be expelled through a nozzle at high velocity. Liquid propellants are preferred over solid propellants where it is necessary to vary thrust during flight. Liquid propellants are classified as bipropellants and monopropellants and the latter are either a single compound or mixtures of compounds. Monopropellant systems are advantageous in that they require only one tank, one pump, one nozzle, one fuel line, one set of controls, etc. Furthermore, no mixing or proportioning system is required.

The principal elements of a rocket motor utilizing a liquid fuel comprise a combustion chamber, exhaust nozzle, an injection system, and propellant control valves. The propellant gases are produced in the combustion chamber at pressures governed by the chemical characteristics of the propellant, its rate of consumption, and the cross-sectional area of the nozzle throat. The gases are ejected into the atmosphere through the nozzle with supersonic velocity. The function of the nozzle is to convert the pressure of the propellant gases into kinetic energy. The reaction of the discharge of the propellant gases constitute the thrust developed by the rocket motor.

The following are objects of this invention.

An object of this invention is to provide a novel two-component monopropellant combination. A further object of this invention is to provide a method for operating rocket motors.

Other aspects, objects, and advantages of this invention will be apparent to one skilled in the art upon reading this disclosure.

In accordance with the invention there are provided novel two-component monopropellant compositions, suitable for use according to the method of the invention in rocket motors and the like. Broadly speaking, the invention comprises the use of an amine nitrate and a suitable oxidant as a two-component monopropellant.

Thus according to the invention there is provided a two-component monopropellant comprising a mixture of (1) an oxidant and (2) an amine nitrate selected from the group consisting of piperidine nitrate, pyridine nitrate, 2-methylpyridine nitrate, and amine nitrates characterized by a formula selected from the group consisting of



and



wherein: each  $R_1$  is selected from the group consisting of acyclic, alicyclic, and aromatic hydrocarbon radicals con-

taining from 1 to 8 carbon atoms, and hydrogen; and  $R_2$  is selected from the group consisting of

- (a) Alkylene, alkenylene, and alkynylene hydrocarbon radicals containing from 1 to 8 carbon atoms, and  
 5 (b)  $\pm R_3-X\{yR_3-$  radicals wherein each  $R_3$  is an alkylene radical containing from 1 to 4 carbon atoms, and  $X$  is selected from the group consisting of oxygen, sulfur, and



and



20 radicals wherein  $R_1$  is defined as above,  $y$  is an integer of from 1 to 3,  $z$  is an integer of from 1 to 3, and  $n$  is an integer from 1 to 5;

25 the total number of carbon atoms in the molecule does not exceed 40, and the total number of amine nitrogen atoms in the molecule does not exceed 10.

Examples of amine nitrates suitable for use in the practice of the invention include, among others, the following:

- 30 methylamine nitrate;  
 dimethylamine nitrate;  
 trimethylamine nitrate;  
 mono-, di- or triethylamine nitrate;  
 propylamine nitrate;  
 35 isopropylamine nitrate;  
 tertiary butylamine nitrate;  
 isobutylamine nitrate;  
 $N,N,N',N'$ -tetramethylbutane-1,2-diamine dinitrate;  
 $N,N,N',N'$ -tetraethylpentane-1,3-diamine dinitrate;  
 $N,N,N',N'$ -tetramethylhexane-3,4-diamine dinitrate;  
 40 pyridine nitrate;  
 2-methylpyridine nitrate;  
 piperidine nitrate;  
 tri-n-octylamine nitrate;  
 45  $N,N$ -dimethyl-2-butetyl-1-amine nitrate;  
 $N$ -ethyl-2-butynylamine-nitrate;  
 $N$ -isopropyl-3,5-dimethylcyclohexylamine nitrate;  
 4-cyclohexenylamine nitrate;  
 $N,N$ -dimethylaniline nitrate;  
 triphenylamine nitrate;  
 $N,N$ -di-n-octyl-p-tolylamine nitrate;  
 $\alpha$ -methylbenzylamine nitrate;  
 diisopropylamine nitrate;  
 $N,N,N',N'$ -tetramethylethane-1,2-diamine dinitrate;  
 $N,N,N',N'$ -tetramethylpropane-1,2-diamine dinitrate;  
 $N,N,N',N'$ -tetramethylbutane-1,3-diamine dinitrate;  
 50 ethane-1,2-diamine dinitrite;  
 $N,N,N',N'$ -tetramethyl-2-butyne-1,4-diamine dinitrate;  
 $N,N,N',N'$ -tetraethylmethane-1,2-diamine dinitrate;  
 $N,N,N',N'$ -tetramethylbutane-1,4-diamine dinitrate;  
 $N,N,N',N'$ -tetramethyloctene-4,8-diamine dinitrate;  
 $N$ -phenyl- $N$ '-n-octylethylene-1,2-diamine mononitrate;  
 $N,N,N',N'$ -tetra-n-octylolctane-1,2-diamine dinitrate;  
 $N,N,N',N'$ -tetracyclohexylhexane-2,5-diamine dinitrate;  
 $N,N'$ -di-p-tolylpropane-1,3-diamine mononitrate;  
 $N$ - $\alpha$ -methylbenzyl-2-butene-1,4-diamine mononitrate;  
 $N,N'$ -dicyclohexenylethane-1,2-diamine dinitrate;  
 $N,N,N',N'$ -tetramethyl-2-butene-1,4-diamine dinitrate;  
 $N,N,N',N'$ -tetraethylpropane-1,3-diamine dinitrate;  
 $N$ -2,4-dimethylcyclohexyl- $N$ '-n-octyl-n-octane-1,8-di-  
 65 amine dinitrate;  
 $N$ -1,4-diamino-2-butene dinitrate;

N,N,N',N'-tetraphenyl-n-3-octene-1,3-diamine dinitrate; N,N'-di(2-ethylhexyl)2-butene-1,4-diamine mononitrate; N,N,N'-tri-n-propenyl-2-butene-1,3-diamine dinitrate; N-cyclohexyl-N'-cyclohexenylpropane-1,3-diamine mononitrate; N,N,N',N'-tetraethyl-4-octyne-1,8-diamine dinitrate; N,N'-dimethylethylene-1,2-diamine dinitrate; N,N'-di(2,4-dimethylphenyl)-2-butyne-1,4-diamine mononitrate; N,N-dicyclohexyl-2-pentyne-1,5-diamine dinitrate; N,N,N'-tri-n-butenyl-2-butene-1,4-diamine mononitrate; bis-(N,N-dimethylaminoethyl)ether dinitrate; bis(N,N-di-n-octylamino-n-butyl)ether mononitrate; N-cyclohexylaminopropyl N-phenylaminopropyl ether dinitrate; N-2-ethylphenylaminoethyl amino-n-butyl ether dinitrate; bis(amino-n-butyl)ether dinitrate; bis(N,N-di-2-ethylcyclohexylamino-n-butyl)thioether dinitrate; bis(aminoethyl)thioether mononitrate; bis(N,N-dimethylaminoethyl)thioether dinitrate; N,N,N',N'-tetramethyl-1,3-diamino-2-propanol dinitrate; N,N,N',N'-tetraethyl-1,3-diamino-2-propanol dinitrate; N,N'-diphenyl-1,9-diamino-5-nonanol mononitrate; N,N,N',N'-tri-2-ethylcyclohexyl-1,4-diamino-2-butanol dinitrate; N,N-di-(2,4-dimethylphenyl)-1,3-diamino-2-propanol mononitrate; N,N'-dicyclohexyl-1,4-diamino-2-butanol dinitrate; N,N,N',N'-tetra-n-propenyl-1,6-diamino-4-hexanol mononitrate; N,N'-dimethylethane-1,2-diamine dinitrate; N,N,N',N',N''-pentamethyldiethylenetriamine trinitrate; N,N',N''-tricyclohexyldiethylenetriamine dinitrate; N,N,N',N'',N''-pentaphenylidibutylideneetriamine trinitrate; N,N-di-p-tolyldipropylideneetriamine mononitrate; N,N,N'-tri-n-octyldiethylenetriamine trinitrate; N,N,N',N'',N''-penta-2-ethylbutyldiethylene triamine dinitrate; N,N,N''-tri-2-ethylcyclohexyldiethylenetriamine trinitrate; diethylene triamine trinitrate; N,N,N',N'',N''-hexamethylpropane-1,2,3-triamine trinitrate; N,N,N'',N''-tetra(2-ethylphenyl)butane-1,2,3,4-tetramine dinitrate; N,N-di(2,4-dimethylcyclohexyl)pentane-1,3,5-triamine trinitrate; N,N,N',N'',N''-hexa-2-butenylpropane-1,2,3-triamine mononitrate; propane-1,2,3-triamine trinitrate; N<sub>1</sub>,N<sub>1</sub>,N<sub>2</sub>,N<sub>2</sub>,N<sub>3</sub>,N<sub>3</sub>,N<sub>4</sub>,N<sub>4</sub>,N<sub>5</sub>,N<sub>5</sub>-decamethylpentane, 1,2,3,4,5-pentamine pentanitrate, N<sub>1</sub>,N<sub>2</sub>,N<sub>3</sub>,N<sub>4</sub>,N<sub>5</sub>-pentaethyltetraethylenepentamine trinitrate; N,N,N',N'-tetra-n-propyl-2,4,6-trihydroxyheptane-1,7-diamine dinitrate; N,N,N',N'-tetramethyl-3,6-dioxaoctane-1,8-diamine dinitrate, and 2,4,6-trithiaheptane-1,7-diamine mononitrate, and 1,2,3,4,6,7,8,10,11,12-deca(N-methylamino)dodecane pentanitrate.

The amine nitrates described above are oxygen deficient and consequently the fuel compositions of my invention require an oxidant. Suitable oxidants that can be used in the two-component monopropellant compositions include anhydrous nitric acid, nitric acid (red and white fuming), hydrogen peroxide, and the liquid nitro substituted aliphatic hydrocarbons such as nitro methane, dinitromethane, trinitromethane, tetrinitromethane, nitroethane, di-nitroethane, trinitroethane, pentanitropropane, and the like.

Nitric acid is the presently preferred oxidant for use in the practice of the invention. Since water tends to retard

combustion of the acid with the fuel, the nitric acid is preferably substantially free of water. Thus, the presently most preferred oxidant is anhydrous nitric acid. However, other more dilute nitric acids can be used in the practice of the invention. White fuming nitric acids and red fuming nitric acids of varying concentrations are available commercially, and all are useful in the practice of this invention. White fuming nitric acid usually contains about 90 to 99 weight percent HNO<sub>3</sub>, from 0 to 2 weight percent NO<sub>2</sub>, and up to about 10 weight percent water. Red fuming nitric acid usually contains about 70 to 90 weight percent HNO<sub>3</sub>, from 2 to 25 weight percent NO<sub>2</sub>, and up to about 10 weight percent water. Of course, mixtures of the above described acids can be employed to give an acid having any intermediate composition, and all are useful in the practice of this invention. Thus, it has been found that nitric acids of all types containing at least about 70 weight percent HNO<sub>3</sub> are useful as an oxidant in the practice of the invention.

The monopropellants used in the present invention will be preferably near stoichiometric mixtures of oxidant and amine nitrate. The ratio of fuel component to oxidant can be in the range of 0.75 to 1.25 times that of the stoichiometric amount. A slightly fuel-rich mixture is usually required to give an optimum rocket motor performance. Amine nitrates can be prepared by several methods. One method is to react an amine with nitric acid. Another method which can be employed is to form a salt of the amine, such as a hydrochloride or an acetate, and then react the amine salt with nitric acid. When amine nitrates are to be prepared by the direct reaction of an amine with nitric acid, and when nitric acid is to be employed as the oxidant in the monopropellants of the invention, said amine nitrates can be prepared in situ by adding the amine to the calculated amount of nitric acid. However, the normally preferred procedure is to admix the amine nitrate, prepared by any suitable method, with nitric acid or another suitable oxidant in the desired ratio at some time prior to use. The length of storage prior to use will depend upon the storage stability of the particular monopropellant composition being employed as will be shown hereinafter.

The amine nitrate-nitric acid two-component monopropellants of the present invention can be conveniently ignited by contacting a stream of the monopropellant with a stream of a hypergol such as pyrrole. Any material which is hypergolic when mixed with nitric acid can be used. Other materials hypergolic with nitric acid such as N,N,N',N'-tetramethyl propane-1,3-diamine; N,N,N',N'-tetramethyl propene-1,3-diamine; furfuryl alcohol; ethylene diamine; etc., can also be used to ignite the two-component monopropellant. These hypergols are simultaneously injected into the combustion chamber with the two-component monopropellant to ignite the monopropellant. After the two-component monopropellant is ignited, the flow of hypergol is stopped. A temperature-sensitive element, a time mechanism or other means can be used to terminate the flow of the hypergol. The other two-component monopropellant compositions of the present invention can be ignited by other means such as, for example, by an electric igniter which, of course, can also be used for amine nitrate-nitric acid mixtures. Suitable apparatus is shown in my copending application, Serial No. 465,957, filed November 1, 1955.

#### EXAMPLE I

A number of runs were made in which polyamine compounds were reacted with nitric acid to form the corresponding amine nitrates. These runs were carried out according to the following procedure.

An amount of the pure polyamine compound was charged to a flask, after which an amount of aqueous nitric acid was charged slowly to said flask by means

of a dropping funnel. The temperature of the flask contents was maintained within the range of from 0 to 10° C. by means of an ice bath and by adjusting the rate of addition of the nitric acid to keep the temperature of the reaction mass below 10° C. During the addition of the nitric acid, the flask contents were stirred vigorously. After the nitric acid had been charged, the flask contents were stirred for several minutes to insure complete reaction, after which said flask contents were poured into approximately 5 times its volume of chilled acetone (-10 to -25° C.). The amine nitrate precipitated out. This precipitate was recovered by filtration, washed with cold acetone or ether, and dried in a vacuum desiccator at room temperature. The melting point and stability of the amine nitrate were then determined. None of the amine nitrates which were prepared were found to be shock sensitive to the blow of a hammer. The results of these runs are given below in Table I.

TABLE I

| Run No. | Amine Charged                                                                     | Mols Nitric Acid Charged | Percent Aqueous Acid (Wt. Percent $\text{HNO}_3$ ) | Mols Amine Charged | Yield of Amine Nitrate, Percent | M.P. of Amine Nitrate, °C. |
|---------|-----------------------------------------------------------------------------------|--------------------------|----------------------------------------------------|--------------------|---------------------------------|----------------------------|
| 1       | $\text{N},\text{N},\text{N}',\text{N}'\text{-tetramethyllethane-1,2-diamine}$     | 0.606                    | 40.5                                               | 0.275              | 96.3                            | 220-221                    |
| 2       | $\text{N},\text{N},\text{N}',\text{N}'\text{-tetramethylpropane-1,2-diamine}$     | 0.606                    | 33.4                                               | 0.275              | 92.3                            | 177-179                    |
| 3       | $\text{N},\text{N},\text{N}',\text{N}'\text{-tetramethylbutane-1,3-diamine}$      | 0.606                    | 40.5                                               | 0.275              | 95.0                            | 115-116                    |
| 3a      | $\text{N},\text{N},\text{N}',\text{N}'\text{-tetramethylbutane-1,3-diamine}$      | 1.19                     | 70.0                                               | 0.578              | 97.0                            | 115-116                    |
| 4       | $\text{N},\text{N},\text{N}',\text{N}'\text{-tetramethyl-2-butyne-1,4-diamine}$   | 0.6                      | 41.0                                               | 0.285              | 96.4                            | 145-146                    |
| 5       | $\text{N},\text{N},\text{N}',\text{N}'\text{-tetraethyllethane-1,2-diamine}$      | 0.6                      | 41.0                                               | 0.285              | 76.5                            | 142-143                    |
| 6       | $\text{N},\text{N},\text{N}',\text{N}'\text{-tetramethylbutane-1,4-diamine}$      | 0.43                     | 70.0                                               | 0.208              | 98.7                            | 173-174                    |
| 7       | $\text{N},\text{N},\text{N}',\text{N}'\text{-tetramethylbutane-1,2-diamine}$      | 0.40                     | 70.0                                               | 0.183              | 94.3                            | 173-174                    |
| 8       | $\text{Bis}(\text{N},\text{N}\text{-dimethylaminoethyl})\text{ether}$             | 0.51                     | 70.0                                               | <sup>1</sup> 0.25  | 72.0                            | 88-93                      |
| 9       | $\text{N},\text{N},\text{N}',\text{N}'\text{-tetramethyl-1,3-diamino-2-propanol}$ | 0.51                     | 70.0                                               | 0.25               | 85.2                            | 120-124                    |
| 10      | $\text{N},\text{N},\text{N}',\text{N}'\text{-tetraethyl-1,3-diamino-2-propanol}$  | 0.51                     | 70.0                                               | 0.25               | 91.2                            | 113-114                    |
| 11      | $\text{N},\text{N},\text{N}',\text{N}'\text{-pentamethylideneetriamine}$          | 0.70                     | 70.0                                               | 0.28               | 80.0                            | 162-163                    |
| 12      | $\text{N},\text{N},\text{N}',\text{N}'\text{-hexamethylpropane-1,2,3-triamine}$   | 0.53                     | 70.0                                               | 0.173              | 65.3                            | 104-106                    |
| 13      | $\text{N},\text{N}\text{-dimethylethylene-1,2-diamine}$                           | 0.605                    | 60.0                                               | 0.5                | <sup>(2)</sup> 125              |                            |
| 14      | $\text{N},\text{N},\text{N}',\text{N}'\text{-tetramethyl-2-butene-1,4-diamine}$   | 0.44                     | 70.0                                               | 0.21               | 88.8                            | 179-180                    |
| 15      | $\text{N},\text{N},\text{N}',\text{N}'\text{-tetraethylpropane-1,3-diamine}$      | 0.42                     | 70.0                                               | 0.2                | 97.0                            | 157.5-159.5                |

<sup>1</sup> In this run, the amine was dissolved in an equal volume of acetone.

<sup>2</sup> Not recorded.

Since the liquid propellants of the invention will be used at high altitudes or, in some instances may be stored in arctic regions, temperatures in the order of -40° F. will frequently be encountered when employing the monopropellant of the present invention. Thus, preferred monopropellants of this invention are those mixtures of amine nitrate and oxidant in which the solubility of the amine nitrate in the oxidant at -40° F. is greater than the percentage of amine nitrate required in the fuel-oxidant mixture for stoichiometric combustion to  $\text{N}_2$ ,  $\text{H}_2\text{O}$ , and  $\text{CO}_2$ . Some examples of fuel-oxidant mixtures which meet this requirement, and are thus preferred, are mixtures of white fuming nitric acid with:  $\text{N},\text{N},\text{N}',\text{N}'\text{-tetramethylpropane-1,2-diamine}$  dinitrate;  $\text{N},\text{N},\text{N}',\text{N}'\text{-tetramethylbutane-1,3-diamine}$  dinitrate;  $\text{N},\text{N},\text{N}',\text{N}'\text{-tetraethyllethane-1,2-diamine}$  dinitrate;  $\text{N},\text{N},\text{N}',\text{N}'\text{-tetraethyl-1,3-diamino-2-propanol}$  dinitrate;  $\text{N},\text{N},\text{N}',\text{N}'\text{-pentamethylideneetriamine}$  trinitrate;  $\text{N},\text{N},\text{N}',\text{N}'\text{-hexamethylpropane-1,2,3-triamine}$  trinitrate;  $\text{N},\text{N}\text{-dimethylethylene-1,2-diamine}$  dinitrate; and  $\text{N},\text{N},\text{N}',\text{N}'\text{-tetramethylpropane-1,3-diamine}$  dinitrate.

#### EXAMPLE II

The amine nitrates which were prepared as described in Example I were dissolved in white fuming nitric acid (WFNA) and the solubilities in weight percent of these compounds in the solvent were determined at -40° F. The white fuming nitric acid used had a composition of 92 weight percent  $\text{HNO}_3$  and 8 weight percent water. In addition, the weight percent of amine nitrate required in a solution of the amine nitrate in white fuming nitric acid for stoichiometric combustion to  $\text{H}_2\text{O}$ ,  $\text{CO}_2$ , and  $\text{N}_2$  was calculated. The solubilities and calculated stoichiometric requirements are tabulated below as Table II.

TABLE II

| 5  | Amine Nitrate from Run—of Ex. I | Solubility (Wt. percent of Amine Nitrate in WFNA at -40° F.) | Calculated Wt. percent of Amine Nitrate for Stoichiometric Ratio of Nitrate and WFNA |
|----|---------------------------------|--------------------------------------------------------------|--------------------------------------------------------------------------------------|
| 1  |                                 | 35.1                                                         | 37.1                                                                                 |
| 2  |                                 | 44.5                                                         | 34.2                                                                                 |
| 3  |                                 | 54.3                                                         | 32.0                                                                                 |
| 4  |                                 | 33.5                                                         | 35.1                                                                                 |
| 5  |                                 | 45.0                                                         | 28.7                                                                                 |
| 6  |                                 | 19.3                                                         | 32.0                                                                                 |
| 7  |                                 | 24.1                                                         | 32.0                                                                                 |
| 8  |                                 | Too hygroscopic, could not be determined accurately.         |                                                                                      |
| 9  |                                 | 33.8                                                         | 36.9                                                                                 |
| 10 |                                 | 35.9                                                         | 29.0                                                                                 |
| 11 |                                 | 43.3                                                         | 37.5                                                                                 |
| 12 |                                 | 38.7                                                         | 37.5                                                                                 |
| 13 |                                 | 38.5                                                         | 38.2                                                                                 |
| 14 |                                 | 18.5                                                         | 32.8                                                                                 |
| 15 |                                 | 35.5                                                         | 34.2                                                                                 |

#### EXAMPLE III

The compound from Run 3 of Example I,  $\text{N},\text{N},\text{N}',\text{N}'\text{-tetramethylbutane-1,3-diamine}$  dinitrate, was dissolved in white fuming nitric acid (identical to that of Example II) in stoichiometric proportion (calculated to  $\text{N}_2$ ,  $\text{H}_2\text{O}$ , and  $\text{CO}_2$ ) plus 5 percent excess of the amine nitrate. This solution was charged to a test tube and placed in an optical bomb under a nitrogen atmosphere. The amine nitrate-WFNA solution was then ignited by means of a high resistance electrical wire, and the time required for a 2" long section of the tube contents to be burned was recorded. The burning rate in inches per second for the propellant mixture was then calculated. Two runs were carried out in this manner, one at a bomb pressure of 300 p.s.i.g., and the other at a bomb pressure of 600 p.s.i.g. At 300 p.s.i.g., the burning rate was found to be 0.08" per second while the burning rate at 600 p.s.i.g., was found to be 0.13" per second.

The freezing point of the above WFNA-amine nitrate mixture was found to be <-52° C., while the refractive index at 25.5° C. was found to be 1.443. The measured density of this mixture was 1.447 (at 26.5° C.).

#### EXAMPLE IV

Performance characteristics of a two-component monopropellant comprising a stoichiometric mixture of methylamine nitrate with nitric acid and dinitromethane are presented in Table I.

TABLE I

| 70                   | Fuel  | Exhaust Temp.,° K | C* Ft./sec. | I Sec. sp. 300 p.s.i. |
|----------------------|-------|-------------------|-------------|-----------------------|
| Methylamine nitrate: |       |                   |             |                       |
| + $\text{HNO}_3$     | 2,923 | 5,030             | 220         |                       |
| + Dinitromethane     | 3,380 | 5,178             | 226         |                       |

As can be seen from the data, stoichiometric mixtures of the fuel give a good performance, although, as stated, a richer mixture than the stoichiometric ratio can be used to achieve optimum specific impulse.

## EXAMPLE V

## Preparation of anhydrous nitric acid

To a 5-liter, 3-necked, round bottom flask there were charged 1.5 liters of WFNA (commercial grade—92% nitric acid, 8% water, and containing a trace of  $\text{NO}_2$ ). Fifteen grams of urea were added to the flask and dry air was bubbled through the mixture at 60° C. for 3 hours or until the presence of nitrogen dioxide as indicated by red coloring was removed. The mixture was cooled to room temperature and 550 milliliters of concentrated sulfuric acid was added. The 3-necked flask was then fitted with a thermometer and a jacketed distillation column which was cooled with ice water. Heat was gradually applied as dry air was bubbled through the mixture. A

51% yield of essentially anhydrous nitric acid which distilled at 45–50° C. was obtained. It was found that anhydrous nitric acid could be stored at —17.7° C. (0° F.) or frozen solid at Dry Ice temperatures for at least 60 days without the formation of the red nitrogen dioxide coloration which would indicate some decomposition.

As disclosed and claimed in copending application Serial No. 678,244, filed by R. C. Doss on Aug. 14, 1957, it has been found that certain materials when added to nitric acid stabilize said acid against the evolution of various nitrogen oxides. Said stabilizing materials include urea and acetamide and ammonium fluoride. Table III given below shows burning rates and other properties of a number of the monopropellants of the present invention in some of which a stabilizing additive has been incorporated. A comparison of the results shows that while said additives render the monopropellant more stable with respect to temperature, they have no appreciable effect on said burning rates.

TABLE III

|                                                                                                                                | (1)<br>N,N,N',N'-tetramethyl-<br>ethane-1,2-diamine dinitrate+ | (2)<br>N,N,N',N'-tetramethyl-<br>propane-1,3-diamine<br>dinitrate+ | (3)<br>N,N,N',N'-tetramethyl-<br>propane-1,2-diamine dini-<br>trate | (4)<br>N,N,N',N'-tetramethyl-<br>butane-1,4-diamine<br>dinitrate+ |                   |                                |
|--------------------------------------------------------------------------------------------------------------------------------|----------------------------------------------------------------|--------------------------------------------------------------------|---------------------------------------------------------------------|-------------------------------------------------------------------|-------------------|--------------------------------|
|                                                                                                                                | 1.4%<br>Acetamide                                              | 1.4%<br>Acetamide                                                  | 0.79%<br>$\text{NH}_4\text{F}$                                      | 1.4%<br>Acetamide                                                 | 1.4%<br>Acetamide | 0.79%<br>$\text{HN}_4\text{F}$ |
| Properties of Unmixed Amine Nitrates:                                                                                          |                                                                |                                                                    |                                                                     |                                                                   |                   |                                |
| Impact Sensitivity, inch pounds.....                                                                                           | >120                                                           | >120                                                               |                                                                     | >120                                                              | >120              |                                |
| Wt. percent Solubility in Anh. $\text{HNO}_3$ :                                                                                |                                                                |                                                                    |                                                                     |                                                                   |                   |                                |
| 75° F.....                                                                                                                     |                                                                |                                                                    |                                                                     |                                                                   |                   |                                |
| 32° F.....                                                                                                                     | 44.5                                                           | 46.6                                                               |                                                                     | 57.6                                                              | 47.4              |                                |
| —40° F.....                                                                                                                    | 32.4                                                           | 42.3                                                               |                                                                     | 53.8                                                              | 38.5              |                                |
| Properties of Stoichiometric Mixtures of Amine Nitrates and Anhydrous Nitric Acid Plus Indicated Amounts of Stabilizing Agent: |                                                                |                                                                    |                                                                     |                                                                   |                   |                                |
| Wt. percent Salt Content of Mixture.....                                                                                       |                                                                |                                                                    |                                                                     |                                                                   |                   |                                |
| Oxidizer to Fuel Ratio, WA/WS <sup>a</sup> .....                                                                               |                                                                |                                                                    |                                                                     |                                                                   |                   |                                |
| Freezing Point, °F.....                                                                                                        |                                                                |                                                                    |                                                                     |                                                                   |                   |                                |
| Mixture Density, g./ml. at 20/4°.....                                                                                          |                                                                |                                                                    |                                                                     |                                                                   |                   |                                |
| Storage Stability at 140° F., hrs.....                                                                                         |                                                                |                                                                    |                                                                     |                                                                   |                   |                                |
| Burning Rate, inches/sec. at—                                                                                                  |                                                                |                                                                    |                                                                     |                                                                   |                   |                                |
| 200 p.s.i.....                                                                                                                 |                                                                |                                                                    |                                                                     |                                                                   |                   |                                |
| 300 p.s.i.....                                                                                                                 |                                                                |                                                                    |                                                                     |                                                                   |                   |                                |
| 400 p.s.i.....                                                                                                                 |                                                                |                                                                    |                                                                     |                                                                   |                   |                                |
| 600 p.s.i.....                                                                                                                 |                                                                |                                                                    |                                                                     |                                                                   |                   |                                |
| Calculated Performance Values of Mixtures of Amine Nitrates and Anhydrous Nitric Acid: <sup>b</sup>                            |                                                                |                                                                    |                                                                     |                                                                   |                   |                                |
| Maximum Specific Impulse, lb.-sec./lb.....                                                                                     | 223.5                                                          | 222.0                                                              |                                                                     | 222.4                                                             | 223.0             |                                |
| Optimum Mixture Ratio, WA/WS.....                                                                                              | 1.12                                                           | 1.30                                                               |                                                                     | 1.30                                                              | 1.44              |                                |

|                                                                                                                                | (5)<br>N,N,N',N'-tetramethyl-butane-1,3-diamine dinitrate + |                |                             |                                               | (6)<br>N,N,N',N'-tetramethyl-<br>butane-1,2-diamine dini-<br>trate + 1.4% Acetamide |
|--------------------------------------------------------------------------------------------------------------------------------|-------------------------------------------------------------|----------------|-----------------------------|-----------------------------------------------|-------------------------------------------------------------------------------------|
|                                                                                                                                | No. Add.                                                    | 1.4% Acetamide | 0.79% $\text{NH}_4\text{F}$ | 1.4% Acetamide<br>0.79% $\text{NH}_4\text{F}$ |                                                                                     |
| Properties of Unmixed Amine Nitrates:                                                                                          |                                                             |                |                             |                                               | >120                                                                                |
| Impact Sensitivity, inch pounds.....                                                                                           |                                                             | >120           |                             |                                               |                                                                                     |
| Wt. Percent Solubility in Anh. $\text{HNO}_3$ :                                                                                |                                                             |                |                             |                                               |                                                                                     |
| 75° F.....                                                                                                                     |                                                             |                |                             |                                               |                                                                                     |
| 32° F.....                                                                                                                     |                                                             | 79.8           |                             |                                               | 48.7                                                                                |
| —40° F.....                                                                                                                    |                                                             | 61.2           |                             |                                               | 41.6                                                                                |
| Properties of Stoichiometric Mixtures of Amine Nitrates and Anhydrous Nitric Acid Plus Indicated Amounts of Stabilizing Agent: |                                                             |                |                             |                                               | 32.7                                                                                |
| Wt. Percent Salt Content of Mixture.....                                                                                       |                                                             |                |                             |                                               |                                                                                     |
| Oxidizer to Fuel Ratio, WA/WS <sup>a</sup> .....                                                                               |                                                             |                |                             |                                               |                                                                                     |
| Freezing Point, °F.....                                                                                                        |                                                             |                |                             |                                               |                                                                                     |
| Mixture Density, g./ml. at 20/4°.....                                                                                          |                                                             |                |                             |                                               |                                                                                     |
| Storage Stability at 140° F., hrs.....                                                                                         |                                                             |                |                             |                                               |                                                                                     |
| Burning Rate, inches/sec. at—                                                                                                  |                                                             |                |                             |                                               |                                                                                     |
| 200 p.s.i.....                                                                                                                 |                                                             | 0.070          | 0.063                       | 0.068                                         |                                                                                     |
| 300 p.s.i.....                                                                                                                 |                                                             | 0.102          | 0.172                       | 0.183                                         |                                                                                     |
| 400 p.s.i.....                                                                                                                 |                                                             | 0.241          | 0.208                       | 0.228                                         | 0.067                                                                               |
| 600 p.s.i.....                                                                                                                 |                                                             | 0.312          | 0.303                       | 0.322                                         | 0.170                                                                               |
| Calculated Performance Values of Mixtures of Amine Nitrates and Anhydrous Nitric Acid: <sup>b</sup>                            |                                                             |                |                             |                                               |                                                                                     |
| Maximum Specific Impulse, lb.-sec./lb.....                                                                                     |                                                             | 223.2          |                             |                                               | 222.22                                                                              |
| Optimum Mixture Ratio, WA/WS.....                                                                                              |                                                             | 1.44           |                             |                                               | 1.44                                                                                |

TABLE III—Continued

|                                                                                                                                | (7)<br>N,N,N',N'-tetramethyl-2-butene-1,4-diamine dinitrate<br>+1.4% Acetamide | (8)<br>N,N,N',N'-tetramethyl-2-butene-1,4-diamine dinitrate<br>+1.4% Acetamide    | (9)<br>N,N,N',N'-tetramethyl ethane-1,2-diamine dinitrate<br>+1.4% Acetamide    |                                                                                     |
|--------------------------------------------------------------------------------------------------------------------------------|--------------------------------------------------------------------------------|-----------------------------------------------------------------------------------|---------------------------------------------------------------------------------|-------------------------------------------------------------------------------------|
| Properties of Unmixed Amine Nitrates:                                                                                          |                                                                                |                                                                                   |                                                                                 |                                                                                     |
| Impact Sensitivity, inch pounds                                                                                                | >120                                                                           | 92                                                                                | >120                                                                            |                                                                                     |
| Wt. percent Solubility in Anh. HNO <sub>3</sub> :                                                                              |                                                                                |                                                                                   |                                                                                 |                                                                                     |
| 75° F                                                                                                                          | 47.6                                                                           | 66.8                                                                              |                                                                                 |                                                                                     |
| 32° F                                                                                                                          | 40.0                                                                           | 56.3                                                                              |                                                                                 |                                                                                     |
| -40° F                                                                                                                         | 31.7                                                                           | 38.8                                                                              |                                                                                 |                                                                                     |
| Properties of Stoichiometric Mixtures of Amine Nitrates and Anhydrous Nitric Acid Plus Indicated Amounts of Stabilizing Agent: |                                                                                |                                                                                   |                                                                                 |                                                                                     |
| Wt. percent Salt Content of Mixture                                                                                            | 34.7                                                                           | 35.7                                                                              | 30.5                                                                            |                                                                                     |
| Oxidizer to Fuel Ratio, WA/SW <sup>a</sup>                                                                                     | 1.881                                                                          | 1.800                                                                             | 2.280                                                                           |                                                                                     |
| Freezing Point, ° F                                                                                                            | b+17.6                                                                         | <-94                                                                              | <-94                                                                            |                                                                                     |
| Mixture Density, g./ml. at 20/4°                                                                                               | 1.418                                                                          | 1.422                                                                             | 1.4114                                                                          |                                                                                     |
| Storage Stability at 140° F., hrs.                                                                                             | 30                                                                             | 6                                                                                 | 37                                                                              |                                                                                     |
| Burning Rate, inches/sec. at—                                                                                                  |                                                                                |                                                                                   |                                                                                 |                                                                                     |
| 200 p.s.i.                                                                                                                     |                                                                                |                                                                                   | 0.061                                                                           |                                                                                     |
| 300 p.s.i.                                                                                                                     |                                                                                |                                                                                   | 0.084                                                                           |                                                                                     |
| 400 p.s.i.                                                                                                                     |                                                                                |                                                                                   | 0.120                                                                           |                                                                                     |
| 600 p.s.i.                                                                                                                     |                                                                                |                                                                                   | 0.192 at 725 p.s.i.                                                             |                                                                                     |
| Calculated Performance Values of Mixtures of Amine Nitrates and Anhydrous Nitric Acid: <sup>f</sup>                            | 223.4                                                                          | 224.7                                                                             | 222.5                                                                           |                                                                                     |
| Maximum Specific Impulse, lb.-sec./lb.                                                                                         | 1.32                                                                           | 1.20                                                                              | 2.69                                                                            |                                                                                     |
| Optimum Mixture Ratio, WA/WS                                                                                                   |                                                                                |                                                                                   |                                                                                 |                                                                                     |
|                                                                                                                                | (10)<br>Bis (dimethyl-amino ethyl)-ether dinitrate+1.4% Acetamide              | (11)<br>N,N,N',N'-tetramethyl-1,3-diamino-2-propanol dinitrate<br>+1.4% Acetamide | (12)<br>N,N,N',N'-tetraethyl-1,3-diamino-2-propane dinitrate<br>+1.4% Acetamide |                                                                                     |
| Properties of Unmixed Amine Nitrates:                                                                                          |                                                                                |                                                                                   |                                                                                 |                                                                                     |
| Impact Sensitivity, inch pounds                                                                                                | >120                                                                           | >120                                                                              | >120                                                                            |                                                                                     |
| Wt. Percent Solubility in Anh. HNO <sub>3</sub> :                                                                              |                                                                                |                                                                                   |                                                                                 |                                                                                     |
| 75° F                                                                                                                          | 79.6                                                                           | 55.8                                                                              |                                                                                 |                                                                                     |
| 32° F                                                                                                                          | 77.3                                                                           | 48.1                                                                              |                                                                                 |                                                                                     |
| -40° F                                                                                                                         | 66.8                                                                           | 35.5                                                                              |                                                                                 |                                                                                     |
| Properties of Stoichiometric Mixtures of Amine Nitrates and Anhydrous Nitric Acid Plus Indicated Amounts of Stabilizing Agent: |                                                                                |                                                                                   |                                                                                 |                                                                                     |
| Wt. Percent Salt Content of Mixture                                                                                            | 36.2                                                                           | 38.9                                                                              | 31.0                                                                            |                                                                                     |
| Oxidizer to Fuel Ratio, WA/WS <sup>a</sup>                                                                                     | 1.761                                                                          | 1.571                                                                             | 2.225                                                                           |                                                                                     |
| Freezing Point, ° F                                                                                                            | <-94                                                                           | <-94                                                                              | <-94                                                                            |                                                                                     |
| Mixture Density, g./ml. at 20/4°                                                                                               | 1.411                                                                          | 1.450                                                                             | 1.414                                                                           |                                                                                     |
| Storage Stability at 140° F., hrs.                                                                                             | 100                                                                            | 5                                                                                 | 16                                                                              |                                                                                     |
| Burning Rate, inches/sec. at—                                                                                                  |                                                                                |                                                                                   |                                                                                 |                                                                                     |
| 200 p.s.i.                                                                                                                     | 0.015                                                                          | 0.034                                                                             | 0.127                                                                           |                                                                                     |
| 300 p.s.i.                                                                                                                     | 0.023                                                                          | 0.059                                                                             | 0.152                                                                           |                                                                                     |
| 400 p.s.i.                                                                                                                     | 0.051                                                                          | 0.093                                                                             | 0.208                                                                           |                                                                                     |
| 600 p.s.i.                                                                                                                     | 0.288                                                                          | 0.212                                                                             | 0.345                                                                           |                                                                                     |
| Calculated Performance Values of Mixtures of Amine Nitrates and Anhydrous Nitric Acid: <sup>f</sup>                            | 220.8                                                                          | 220.2                                                                             | 219.9                                                                           |                                                                                     |
| Maximum Specific Impulse, lb.-sec./lb.                                                                                         | 1.31                                                                           | 1.16                                                                              | 1.69                                                                            |                                                                                     |
| Optimum Mixture Ratio, WA/WS                                                                                                   |                                                                                |                                                                                   |                                                                                 |                                                                                     |
|                                                                                                                                | (13)<br>Hexane-1,6-diamine dinitrate+1.4% Acetamide                            | (14)<br>N,N'-dimethyl-ethane-1,2-diamine dinitrate+1.4% Acetamide                 | (15)<br>N,N'-dimethyl-propane-1,2-diamine dinitrate+1.4% Acetamide              | (16)<br>N,N,N',N"-hexamethyl-1-propane-1,2,3-triamine trinitrate<br>+1.4% Acetamide |
| Properties of Unmixed Amine Nitrates:                                                                                          |                                                                                |                                                                                   |                                                                                 |                                                                                     |
| Impact Sensitivity, inch pounds                                                                                                | >120                                                                           | >120                                                                              | >120                                                                            | >120                                                                                |
| Wt. percent Solubility in Anh. HNO <sub>3</sub> :                                                                              |                                                                                |                                                                                   |                                                                                 |                                                                                     |
| 75° F                                                                                                                          | 82.5                                                                           | 56.1                                                                              | 78.7                                                                            |                                                                                     |
| 32° F                                                                                                                          | 74.0                                                                           | 51.2                                                                              | 70.5                                                                            |                                                                                     |
| -40° F                                                                                                                         | 52.7                                                                           | 46.2                                                                              | 56.0                                                                            |                                                                                     |
| Properties of Stoichiometric Mixtures of Amine Nitrates and Anhydrous Nitric Acid Plus Indicated Amounts of Stabilizing Agent: |                                                                                |                                                                                   |                                                                                 |                                                                                     |
| Wt. percent Salt Content of Mixture                                                                                            | 39.1                                                                           | 48.6                                                                              | 43.1                                                                            | 39.6                                                                                |
| Oxidizer to Fuel Ratio, WA/WS                                                                                                  | 1.555                                                                          | 1.056                                                                             | 1.321                                                                           | 1.523                                                                               |
| Freezing Point, ° F                                                                                                            | >-94                                                                           | 1.451                                                                             |                                                                                 |                                                                                     |
| Mixture Density, g./ml. at 20/4°                                                                                               |                                                                                | 240                                                                               |                                                                                 | 1.4798                                                                              |
| Storage Stability at 140° F., hrs.                                                                                             | 2                                                                              |                                                                                   |                                                                                 | 0                                                                                   |
| Burning Rate, inches/sec. at—                                                                                                  |                                                                                |                                                                                   |                                                                                 |                                                                                     |
| 200 p.s.i.                                                                                                                     |                                                                                | 0.060                                                                             |                                                                                 |                                                                                     |
| 300 p.s.i.                                                                                                                     |                                                                                | 0.146                                                                             |                                                                                 |                                                                                     |
| 400 p.s.i.                                                                                                                     |                                                                                | 0.200                                                                             |                                                                                 |                                                                                     |
| 600 p.s.i.                                                                                                                     |                                                                                | 0.294                                                                             |                                                                                 |                                                                                     |
| Calculated Performance Values of Mixtures of Amine Nitrates and Anhydrous Nitric Acid: <sup>f</sup>                            | 221.0                                                                          | 223.2                                                                             |                                                                                 | 221.8                                                                               |
| Maximum Specific Impulse, lb.-sec./lb.                                                                                         | 1.14                                                                           | 0.72                                                                              |                                                                                 | 1.12                                                                                |
| Optimum Mixture Ratio, WA/WS                                                                                                   |                                                                                |                                                                                   |                                                                                 |                                                                                     |

TABLE III—Continued

|                                                                                                                                | (17)<br>N,N'-diisopropyl-<br>ethane-1,2-diamine<br>dinitrate+No add. | (18)<br>Diisopropylamine<br>nitrate      | (19)<br>Piperidine<br>Nitrate+1.4% Ace-<br>tamide | (20)<br>N,N,N',N'-<br>pentamethyl-di-<br>ethylene-triamine<br>trinitrate |
|--------------------------------------------------------------------------------------------------------------------------------|----------------------------------------------------------------------|------------------------------------------|---------------------------------------------------|--------------------------------------------------------------------------|
| Properties of Unmixed Amine Nitrates:                                                                                          |                                                                      |                                          |                                                   |                                                                          |
| Impact Sensitivity, inch pounds                                                                                                |                                                                      | >120                                     | >120                                              | 62                                                                       |
| Wt. percent Solubility in Anh. HNO <sub>3</sub> :                                                                              |                                                                      |                                          |                                                   |                                                                          |
| 75° F.                                                                                                                         |                                                                      | 75.1                                     |                                                   |                                                                          |
| 32° F.                                                                                                                         |                                                                      | 62.6                                     | 82.6                                              |                                                                          |
| -40° F.                                                                                                                        |                                                                      | 57.2                                     | 61.4                                              |                                                                          |
| Properties of Stoichiometric Mixtures of Amine Nitrates and Anhydrous Nitric Acid Plus Indicated Amounts of Stabilizing Agent: |                                                                      |                                          |                                                   |                                                                          |
| Wt. percent Salt Content of Mixture                                                                                            | 33.8                                                                 | 27.7                                     | 31.1                                              | 39.6                                                                     |
| Oxidizer to Fuel Ratio, WA/WS                                                                                                  | 1.958                                                                | 2.610                                    | 2.216                                             | 1.525                                                                    |
| Freezing Point, ° F.                                                                                                           | >-94                                                                 | <-94                                     | >-94                                              |                                                                          |
| Mixture Density, g./ml. at 20/4 °                                                                                              | 1.4164                                                               | 1.340                                    | 1.400                                             | 1.4817                                                                   |
| Storage Stability at 140° F., hrs.                                                                                             | est. >1 yr.                                                          |                                          | 299                                               |                                                                          |
| Burning Rate, inches/sec. at—                                                                                                  |                                                                      |                                          |                                                   |                                                                          |
| 200 p.s.i.                                                                                                                     |                                                                      | d 0.074                                  |                                                   |                                                                          |
| 300 p.s.i.                                                                                                                     | 0.076                                                                | d 0.055                                  | 0.067                                             |                                                                          |
| 400 p.s.i.                                                                                                                     | 0.101                                                                | d 0.063                                  | 0.098                                             |                                                                          |
| 600 p.s.i.                                                                                                                     | 0.189                                                                | d 0.088                                  |                                                   |                                                                          |
| Calculated Performance Values of Mixtures of Amine Nitrates and Anhydrous Nitric Acid: <sup>f</sup>                            |                                                                      |                                          |                                                   |                                                                          |
| Maximum Specific Impulse, lb.-sec./lb.                                                                                         |                                                                      | 223.3                                    | 222.0                                             | 222.5                                                                    |
| Optimum Mixture Ratio, WA/WS                                                                                                   |                                                                      | 1.94                                     | 1.78                                              | 1.09                                                                     |
|                                                                                                                                | (21)<br>Ethylenediamine<br>dinitrate                                 | (22)<br>Diethylenetriamine<br>trinitrate | (23)<br>Pyridine Nitrate                          | (24)<br>Diallylamine Nitrate                                             |
| Properties of Unmixed Amine Nitrates:                                                                                          |                                                                      |                                          |                                                   |                                                                          |
| Impact Sensitivity, inch pounds                                                                                                | 100                                                                  | 120                                      | >120                                              | >120                                                                     |
| Solubility in Anh. HNO <sub>3</sub> :                                                                                          |                                                                      |                                          |                                                   |                                                                          |
| 75° F.                                                                                                                         | 58.8                                                                 | 52.7                                     |                                                   |                                                                          |
| 32° F.                                                                                                                         | Solid                                                                |                                          |                                                   |                                                                          |
| -40° F.                                                                                                                        | Solid                                                                |                                          |                                                   |                                                                          |
| Properties of Stoichiometric Mixtures of Amine Nitrates and Anhydrous Nitric Acid Plus Indicated Amounts of Stabilizing Agent: |                                                                      |                                          |                                                   |                                                                          |
| Weight Percent Salt Content of Mixture                                                                                         | 71.3                                                                 | 62.4                                     | 36.0                                              | 29.8                                                                     |
| Oxidizer to Fuel Ratio, WA/WS                                                                                                  | 0.402                                                                | 0.603                                    | 1.676                                             | 2.36                                                                     |
| Freezing Point, ° F.                                                                                                           | b +14                                                                | -67 (glass)                              | <-94                                              |                                                                          |
| Mixture Density, g./ml. at 20/4 °                                                                                              | 1.580                                                                | 1.590                                    | 1.441                                             |                                                                          |
| Storage Stability at 140° F., hrs.                                                                                             |                                                                      |                                          |                                                   |                                                                          |
| Burning Rate, inches/sec. at—                                                                                                  |                                                                      |                                          |                                                   |                                                                          |
| 200 p.s.i.                                                                                                                     |                                                                      |                                          |                                                   |                                                                          |
| 300 p.s.i.                                                                                                                     |                                                                      |                                          |                                                   |                                                                          |
| 400 p.s.i.                                                                                                                     |                                                                      |                                          |                                                   |                                                                          |
| 600 p.s.i.                                                                                                                     |                                                                      |                                          |                                                   |                                                                          |
| Calculated Performance Values of Mixtures of Amine Nitrates and Anhydrous Nitric Acid: <sup>f</sup>                            |                                                                      |                                          |                                                   |                                                                          |
| Maximum Specific Impulse, lb.-sec./lb.                                                                                         | • 220.3                                                              | 219.5                                    | 215.2                                             | 221.3                                                                    |
| Optimum Mixture Ratio, WA/WS                                                                                                   | 0.260                                                                | 0.40                                     | 1.22                                              | 1.70                                                                     |

<sup>a</sup> WA/WS=weight of acid/weight of amine salt.<sup>b</sup> The freezing point is given as the temperature at which salt crystals began to precipitate.<sup>c</sup> Densities were determined with a Westphal balance.<sup>d</sup> Determined on 20 wt. percent solution of diisopropylamine nitrate in anhydrous nitric acid.

It is to be realized that the test at 140° is a severe test and the mere fact that some compounds give mixtures which have a low storage stability at 140° F. does not mean that said compounds are not useful in the practice of the invention because, at lower temperatures, mixtures of said compounds with nitric acid to have higher storage stabilities and can be used at lower temperatures in those instances where storage stability is of secondary importance.

The above listed mixtures in Table IV thus represent a select, superior, group of monopropellants. Other considerations such as availability, etc. will enter into the final choice of the most preferred from said select superior group of monopropellants.

As many possible embodiments may be made of this invention without departing from the scope thereof, it is to be understood that all matter herein set forth is to be interpreted as illustrative and not in a limiting sense.

The values for "Storage Stability at 140° F." given in the above Table III were determined by storing 20 milliliters of the acid-salt solution in a 30 milliliter stainless steel bomb immersed in a constant temperature bath. Bomb pressure was then recorded versus time in the storage bath until rupture of a 109 p.s.i. safety disc in the bomb.

Referring to said Table III it will be noted that certain

55      <sup>e</sup> Specific impulse shown is not the maximum. Peak values were not determined.

60      <sup>f</sup> Does not include stabilizer.

of the mixtures listed therein are definitely superior with respect to storage stability, impact sensitivity, burning rate, and solubility in anhydrous nitric acid. Of these properties, storage stability is presently considered to be the most important because the longer the acid-salt solutions can be stored the more useful said mixtures are. Since the monopropellants of the invention may possibly be used or stored under desert conditions, 140° F. was chosen as a reasonable maximum temperature at which to measure storage stability. It will be noted that the following compounds formed mixtures which are definitely superior with respect to storage stability.

TABLE IV

| Number in<br>Table III | Compound                                            |
|------------------------|-----------------------------------------------------|
| 2                      | N,N,N',N'-tetramethylpropane-1,3-diamine dinitrate. |
| 4                      | N,N,N',N'-tetramethylbutane-1,4-diamine dinitrate.  |
| 5                      | N,N,N',N'-tetramethylbutane-1,3-diamine dinitrate.  |
| 6                      | N,N,N',N'-tetramethylbutane-1,2-diamine dinitrate.  |
| 10                     | Bis-(dimethyl-aminoethoxy) ether dinitrate.         |
| 14                     | N,N'-dimethyllethane-1,2-diamine dinitrate.         |
| 18                     | Diisopropyl amine nitrate.                          |
| 19                     | Piperidine nitrate.                                 |

75      It is to be noted that the compounds of Table IV all



## 15

amine nitrates characterized by a formula selected from the group consisting of



and



wherein: each  $\text{R}_1$  is selected from the group consisting of acyclic, alicyclic, and aromatic hydrocarbon radicals containing from 1 to 8 carbon atoms, and hydrogen; and  $\text{R}_2$  is selected from the group consisting of

- (a) alkylene, alkenylene, and alkynylene hydrocarbon radicals containing from 1 to 8 carbon atoms, and
- (b)  $\text{fR}_3-\text{X}_3-\text{R}_3$ —radicals wherein each  $\text{R}_3$  is an alkylene radical containing from 1 to 4 carbon atoms, and  $\text{X}$  is selected from the group consisting of oxygen, sulfur, and



and



radicals wherein  $\text{R}_1$  is defined as above,  $y$  is an integer of from 1 to 3, and  $n$  is an integer of from 1 to 3, and  $n$  is an integer of from 1 to 5;

the total number of carbon atoms in the molecule does not exceed 40, and the total number of amino nitrogen atoms in the molecule does not exceed 10; igniting said mixture by contacting said mixture with a compound hypergolic with said oxidant and selected from the group consisting of pyrrole,  $\text{N},\text{N},\text{N}',\text{N}'$ -tetramethylpropane-1,3-

diamine,  $\text{N},\text{N},\text{N}',\text{N}'$ -tetramethylpropene-1,3-diamine, furfuryl alcohol, and ethylenediamine; discontinuing the flow of said hypergolic compound following ignition of said mixture the ratio of said amine nitrate to said oxidant being in the range of 0.75 to 1.25 times that of the stoichiometric amount; and igniting said mixture.

15. A two-component monopropellant consisting essentially of a mixture of (1) an oxidant selected from the group consisting of nitric acid containing at least about 70 weight percent  $\text{HNO}_3$  and liquid nitro substituted lower alkanes, and (2) an amine nitrate, the ratio of said amine nitrate to said oxidant being in the range of 0.75 to 1.25 times that of the stoichiometric amount.

16. In the method for development of thrust by the combustion of a two-component monopropellant in the combustion chamber of a reaction motor, the steps comprising injecting into said combustion chamber a mixture of (1) an oxidant selected from the group consisting of nitric acid containing at least about 70 weight percent  $\text{HNO}_3$  and liquid nitro substituted lower alkanes, and (2) an amine nitrate, the ratio of said amine nitrate to said oxidant being in the range of 0.75 to 1.25 times that of the stoichiometric amount; and igniting said mixture.

17. A rocket monopropellant which consists of a mixture consisting of approximately stoichiometric proportions of a lower alkyl amine nitrate and nitric acid containing at least 95%  $\text{HNO}_3$  by weight.

## References Cited by the Examiner

## UNITED STATES PATENTS

- |           |       |                             |
|-----------|-------|-----------------------------|
| 2,542,193 | 2/51  | Hannum.                     |
| 2,573,471 | 10/51 | Malina et al. ----- 60-35.4 |
| 2,637,161 | 5/53  | Tschinkel ----- 60-35.4     |

## OTHER REFERENCES

Cottrell et al.: Journal Chemical Society (1951), pp. 1798-1800.

CARL D. QUARFORTH, Primary Examiner.

40 ROGER L. CAMPBELL, LEON D. ROSDOL,  
Examiners.

UNITED STATES PATENT OFFICE  
CERTIFICATE OF CORRECTION

Patent No. 3,212,254

October 19, 1965

Homer M. Fox

It is hereby certified that error appears in the above numbered patent requiring correction and that the said Letters Patent should read as corrected below.

Column 14, line 20, for "+ R<sub>2</sub>-X + y R<sub>3</sub> -" read -- + R<sub>3</sub>-X + y  
R<sub>3</sub> - --; line 54, for the claim reference numeral "1" read --  
7 --; column 15, line 35, for "and n" read -- z --, in italics.

Signed and sealed this 2nd day of August 1966.

(SEAL)

Attest:

ERNEST W. SWIDER  
Attesting Officer

EDWARD J. BRENNER  
Commissioner of Patents